

1

3,600,165

## OPTICAL SENSITISATION OF INORGANIC PHOTOCODUCTORS

Jozef Frans Willems and Albert Lucien Poot, Wilrijk-Antwerp, and Robert Joseph Noe, Mortsel-Antwerp, Belgium, assignors to Gevaert-Agfa N.V., Mortsel, Belgium

No Drawing. Continuation of application Ser. No. 542,753, Apr. 14, 1966. This application Dec. 30, 1969, Ser. No. 888,131

Claims priority, application Great Britain, Apr. 15, 1965, 16,336/65

Int. Cl. G03g 5/08

U.S. CL. 96—1.7

6 Claims

### ABSTRACT OF THE DISCLOSURE

An improved photoconductive material for use in photoconductive recording elements is obtained by treating a conventional inorganic metallic photoconductive compound with a small amount of an organic chelating agent which is adapted to form with the metallic ions of the photoconductive compound a colored chelate of increased light-sensitivity relative to the untreated photoconductive compound. A preferred amount of the chelating compound is 0.001-0.5% by weight of the photoconductive compound. A variety of suitable organic chelating agents are disclosed.

This application is a continuation of Ser. No. 542,753 filed Apr. 14, 1966, now abandoned.

The present invention relates to a recording and reproduction material containing a spectrally sensitized inorganic photoconductive substance and a process for sensitizing said substance.

As inorganic photoconductive substances are known e.g. the oxides, sulphides and selenides of zinc, cadmium, mercury, antimony, bismuth and lead.

The sensitizing agents for inorganic photoconductive substances may be inorganic as well as organic. For instance, for the sensitization of photoconductive zinc oxide mercury sulphide, lead oxide and lead iodide have been proposed as well as organic dyestuffs such as triphenyl methane derivatives, sulphone phthaleins and cyanine dyes of various kinds.

We now have found that an organic compound which can complex a metal ion of the type provided by the inorganic photoconductor and forms a coloured chelate therewith possesses optical sensitizing properties for said inorganic photoconductor.

More particularly several classes of chelating compounds have been found that optically sensitize photoconductive zinc oxide in the absorption range of the formed chelate.

A first class of such compounds is represented by the following general Formula I:



wherein:

R represents a hydrogen atom, an alkyl radical e.g. an alkyl radical having from 1 to 5 carbon atoms, and

Each of Z and Z' represents the atoms necessary for completing a nitrogen-containing five or six-membered ring. Said five or six-membered ring may contain in addition to the nitrogen atom one or more hetero atoms e.g. oxygen, nitrogen, selenium, or sulphur atoms to form a known heterocyclic ring such as those of the thiazole series (e.g. thiazole, 4-methylthiazole, 4-methyl-5-carboxythiazole, 4-phenylthiazole, 5-methylthiazole, 5-phenylthiazole, 4-(p-tolyl)thiazole, 4-(p-bromophenyl)-

2

thiazole, 4,5-dimethylthiazole, 4,5-diphenylthiazole, 4-(2-thienyl)-thiazole, 4-(m-nitrophenyl)thiazole), those of the benzothiazole series (e.g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 6-sulfonic acid benzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, 4,5,6,7-tetrahydrobenzothiazole, 5,6-dimethoxybenzothiazole, 5,6-dioxymethylenebenzothiazole, 5-hydroxybenzothiazole, 6-hydroxybenzothiazole, 5,6-dimethylbenzothiazole), those of the naphthothiazole series (e.g. naphtho[2,1-d]thiazole, naphtho[1,2-d]thiazole, 5-methoxynaphtho[1,2-d]thiazole, 5-ethoxynaphtho[1,2-d]thiazole, 8-methoxynaphtho[2,1-d]thiazole, 7-methoxynaphtho[2,1-d]thiazole), those of the thionaphtheno[7,6-d]thiazole series (e.g. 7-methoxythionaphtheno[7,6-d]thiazole), those of the thiadiazole series (e.g. 4-phenylthiadiazole), those of the oxazole series (e.g. 4-methyloxazole, 5-methyloxazole, 4-phenyloxazole, 4,5-diphenyloxazole, 4-ethyloxazole, 4,5-dimethyloxazole, 5-phenyloxazole), those of the benzoxazole series (e.g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 6-methoxybenzoxazole, 5-hydroxybenzoxazole, 6-hydroxybenzoxazole), those of the naphthoxazole series (e.g. naphtho[2,1-d]oxazole, naphtho[1,2-d]oxazole), those of the selenazole series (e.g. 4-methylselenazole, 4-phenylselenazole), those of the benzoselenazole series (e.g. benzoselenazole, 5-chlorobenzoselenazole, 5-methoxybenzoselenazole, 5-hydroxybenzoselenazole, 4,5,6,7-tetrahydrobenzoselenazole), those of the naphthoselenazole series (e.g. naphtho[2,1-d]selenazole, naphtho[1,2-d]selenazole), those of the 2-quinoline series (e.g. the quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc.), those of the pyrimidine series, those of the quinoxaline series, those of the quinazoline series, those of the 1-phthalazine series, those of the 2-pyridine series (e.g. pyridine, 5-methylpyridine, 3-nitropyridine), those of the benzimidazole series (e.g. 1-ethylbenzimidazole, 1-phenylbenzimidazole, 1-ethyl-5,6-dichlorobenzimidazole, 1-hydroxyethyl-5,6-dichlorobenzimidazole, 1-ethyl-5-chlorobenzimidazole, 1-ethyl-5,6-dibromobenzimidazole, 1-ethyl-5-chloro-6-aminobenzimidazole, 1-ethyl-5-chloro-6-bromobenzimidazole, 1-ethyl-5-phenylbenzimidazole, 1-ethyl-5-fluorobenzimidazole, 1-ethyl-5,6-difluorobenzimidazole, 1-ethyl-5-cyanobenzimidazole, 1-( $\beta$ -acetoxy-ethyl)-5-cyanobenzimidazole, 1-ethyl-5-chloro-6-cyanobenzimidazole, 1-ethyl-5-acetylbenzimidazole, 1-ethyl-5-chloro-6-fluorobenzimidazole, 1-ethyl-5-carboxybenzimidazole, 1-ethyl-7-carboxybenzimidazole, 1-ethyl-5-carbethoxybenzimidazole, 1-ethyl-7-carbethoxybenzimidazole, 1-ethyl-5-sulphamylbenzimidazole, or 1-ethyl-5-N-ethylsulphamylbenzimidazole).

The following is a list of hydrazone compounds to most of which is referred in the examples.

65 (1)



(2)



3



4





10 The preparation of the hydrazone compounds 1, 2 and 5 is described by J. F. Geldard, F. Lions, J. Am. Chem. Soc., 84, 2262-3 (1962).

15 The preparation of the hydrazone compound 23 is described by F. Lions, K. V. Martin, J. Am. Chem. Soc., 80, 3858-65 (1958).

10 The preparation of the hydrazone compound 4 is as follows:

20 0.145 mole of the hydrazone compound 1 is dissolved in 350 ccs. of boiling acetone. To the obtained solution 0.15 mole of zinc sulphate-7-water dissolved in 100 ccs. of water is added whilst stirring.

25 The solution is cooled. The precipitate formed is filtered off, once washed with cold water, twice with ethanol and dried at 100° C.

30 Analysis.—Calculated (percent): C, 34.2; H, 3.37; N, 14.52; S, 8.31. Found (percent): C, 33.92; H, 3.70; N, 14.11; S, 8.87.

35 Hydrazone compound 5 is prepared by heating compound 4 on an oil bath at 220° C. for 3 h.

30 The other hydrazone compounds are prepared according to the following general preparation method:

35 0.025 mole of hydrazino derivative dissolved or suspended in 25 ccs. of ethanol are mixed with 0.025 mole of aldehyde derivative dissolved in 25 ccs. of ethanol.

40 The reaction mixture is refluxed on a boiling water bath for 30 min. After cooling the formed precipitate is sucked off and washed with ethanol and dried. In most cases the obtained product is pure enough so that no further purification is necessary. Only the compounds 20 and 22 are recrystallized from ethylene glycol monomethyl ether.

45 In the following table the starting products, melting point and results of analysis of hydrazone compounds prepared according to the above general preparation method are listed.

| Number | Hydrazino derivative                                                                                                   | Aldehyde derivative                                                                 | Analysis           |             |                        |                        |
|--------|------------------------------------------------------------------------------------------------------------------------|-------------------------------------------------------------------------------------|--------------------|-------------|------------------------|------------------------|
|        |                                                                                                                        |                                                                                     | Melting point, °C. | Elements    | Calc., percent         | Found, percent         |
| 3----- | NH <sub>2</sub> NH <sub>2</sub><br> |  | 195                | C<br>H      | 67.53<br>4.45          | 67.49<br>4.25          |
| 6----- |                                     | Same as above-----                                                                  | 266                | C<br>H<br>S | 59.80<br>3.92<br>11.46 | 60.02<br>4.16<br>11.11 |
| 7----- |                                     | ----do-----                                                                         | 210                | C<br>H<br>S | 64.25<br>4.28<br>11.42 | 64.18<br>4.44<br>11.13 |
| 8----- |                                     | ----do-----                                                                         | >260               | C<br>H      | 65.80<br>4.64          | 65.56<br>4.82          |
| 9----- |                                     | ----do-----                                                                         | >260               | C<br>H      | 67.50<br>4.42          | 67.66<br>4.60          |

| Number  | Hydrazino derivative                                                                | Aldehyde derivative                                                                 | Analysis           |             |                        |
|---------|-------------------------------------------------------------------------------------|-------------------------------------------------------------------------------------|--------------------|-------------|------------------------|
|         |                                                                                     |                                                                                     | Melting point, °C. | Elements    | Calc., percent         |
| 10..... |    |    | 220                | C<br>H      | 68.50<br>4.94          |
| 11..... | Same as above.....                                                                  |    | 244                | C<br>H      | 72.30<br>4.35          |
| 12..... |    | Same as above.....                                                                  | 240                | C<br>H<br>S | 69.10<br>4.24<br>9.70  |
| 13..... |    |    | 260                | C<br>H<br>S | 53.80<br>4.83<br>11.04 |
| 14..... | Same as above.....                                                                  |    | 220                | C<br>H<br>S | 55.25<br>5.26<br>10.52 |
| 15..... | do.....                                                                             |    | 257                | C<br>H<br>S | 60.00<br>4.70<br>9.40  |
| 16..... |   |   | >260               | C<br>H<br>S | 46.70<br>3.00<br>19.18 |
| 17..... |  | Same as above.....                                                                  | 210                | C<br>H<br>S | 55.50<br>3.98<br>19.60 |
| 18..... |  |  | 210                | C<br>H      | 67.50<br>4.42          |
| 19..... |  |  | 215                | C<br>H      | 72.30<br>4.38          |
| 20..... |  |  | 250                | .....       | .....                  |
| 21..... | Same as above.....                                                                  |  | 230                | C<br>H<br>S | 56.60<br>3.84<br>9.45  |
| 22..... | do.....                                                                             |  | 260                | C<br>H<br>S | 60.00<br>3.47<br>8.53  |
| 24..... |  | Same as above.....                                                                  | 210                | C<br>H<br>S | 69.80<br>4.65<br>9.30  |

| Number | Hydrazino derivative | Aldehyde derivative | Melting point, °C. | Analysis    |                        |                        |
|--------|----------------------|---------------------|--------------------|-------------|------------------------|------------------------|
|        |                      |                     |                    | Elements    | Calc., percent         | Found, percent         |
| 25     |                      |                     | 233                | C<br>H<br>S | 70.80<br>4.50<br>8.97  | 71.09<br>4.51<br>9.25  |
| 26     | Same as above        |                     | 246                | C<br>H<br>S | 71.40<br>4.86<br>8.66  | 71.62<br>4.98<br>8.82  |
| 27     | do                   |                     | 240                | C<br>H<br>S | 74.00<br>4.43<br>7.87  | 74.07<br>4.51<br>8.00  |
| 28     |                      |                     | 238                | C<br>H<br>S | 65.30<br>4.76<br>10.89 | 65.60<br>4.58<br>10.88 |
| 29     | Same as above        |                     | 250                | C<br>H<br>S | 66.20<br>5.20<br>10.40 | 66.24<br>5.20<br>10.37 |
| 30     |                      |                     | >260               | C<br>H<br>O | 54.37<br>3.73<br>13.17 | 54.40<br>3.35<br>13.26 |
| 31     |                      |                     | >260               | C<br>H      | 65.80<br>4.06          | 65.72<br>4.39          |
| 32     |                      |                     | 230                | C<br>H<br>S | 50.10<br>3.06<br>8.92  | 50.32<br>3.15<br>9.16  |
| 33     | Same as above        |                     | 250                | C<br>H<br>S | 51.50<br>3.49<br>8.58  | 51.63<br>3.67<br>8.60  |
| 34     | do                   |                     | >260               | C<br>H<br>S | 55.70<br>3.18<br>7.82  | 55.90<br>3.40<br>7.68  |
| 35     |                      |                     | 208                | C<br>H<br>S | 65.30<br>4.76<br>10.90 | 65.56<br>5.06<br>11.32 |
| 37     |                      | Same as above       | 174                | C<br>H      | 64<br>5.34             | 63.96<br>5.39          |

A second class is represented by the following general Formula II:



wherein Z' has the same meaning as described for general Formula I.

As representatives of general Formula II are more particularly mentioned:

70 Compound 38:





13



prepared according to B. Chiswell, F. Lions, Inorg. Chem. 3 (1964) 490.

A seventh class is represented by the following general Formula VII:



wherein:

each of R<sub>4</sub> and R<sub>5</sub> represents alkyl e.g. methyl, aryl e.g. phenyl, or represent together the atoms necessary to close a homocyclic ring, and

Z' has the same meaning as described for general Formula I.

As representatives of general Formula VII are more particularly mentioned:

Compound 50:



Compound 51:



Compound 52:



Compound 53:



Compound 54:



Compound 55:

5



Compound 56:



melting point 190° C.

15



20

melting point 222° C.

The compounds 50-55 are prepared according to B. Chiswell, F. Lions, M. L. Tomlinson Inorg. Chem. 3 (1964) 492. Compound 56 is prepared analogously to the compounds 50-55.

An eighth class is represented by the following general Formula VIII:

30



35

The compounds 57, 58, 59 and 60 wherein R<sub>6</sub> is respectively hydrogen, methyl, carbethoxy and benzoyl are prepared according to B. Eistert, H. Selzer, Chem. Ber. 96 (1963) 314-319.

Further are mentioned chelating compounds for zinc ions containing an aromatic nucleus having in ortho-position to a hydroxyl group a —CH=N— group, a —CO—NH—N=CH— group, a —N=N-aryl group, or a —CH=N—N=CH—aryl group and chelating compounds for zinc ions containing in orthoposition to a carboxyl group an azo group.

Examples of further compounds useful herein are as follows:

50 Compound 61:



melting point 260° C.

which is prepared as follows:

To 0.1 mole of 2-(o-aminophenyl)benzimidazole (Ber. 32, 1465) dissolved in 100 ccs. of ethanol 0.1 mole of salicyl aldehyde is added. The reaction mixture is refluxed for 2 h. on a boiling water bath. The precipitate formed is sucked off and washed with ether. Melting point >260° C. and

Compound 62:



Melting point 213° C.

70

75

The sensitizing compounds are preferably used in dissolved form to sensitize the inorganic photoconductor which is normally used in dispersed form in a solution or dispersion of a binder. They may be mixed beforehand, for example dissolved in dimethylformamide with the photo conductor e.g. zinc oxide. The sensitizing compound is then adsorbed on the photoconductor grains and can complex metal ions provided by the photoconductor. The sensitized photoconductor thus treated is then mixed with a suitable binder, whereupon the whole composition can be coated on a suitable base material.

The sensitizing compounds may also be used in complexed form as can be seen e.g. in Example 2. Thus it is not absolutely necessary to treat the photoconductive substances with the sensitizing compounds in non-complexed form, although the sensitizing treatment with the compounds in non-complexed form is preferred.

The sensitizing compounds used in the present invention are preferably applied in combination with an acid to produce metal ions; preferably the acid compounds described in Belgian patent specification 612,102 filed Dec. 29, 1961 by Gevaert Photo-Producten N.V. which increases the dark resistivity of photoconductive zinc oxide are used. Of course the spectral sensitivity of photoconductive recording layers according to the present invention may be further modified by sensitizing compounds other than those described herein.

Combinations with other optical sensitizing compounds may be applied in order to make the recording layer sensitive for the whole range of the visible spectrum, so that the recording layer becomes suitable for multicolour reproduction.

The quantitative ratio of photoconductor to sensitizing agent may vary within wide limits and depends on the effect desired; the amount of sensitizing agent may for instance vary between 0.001 and 0.5 percent based on the weight of photoconductor. Representatives of sensitizing compounds which are very active can be chosen in Table 2 of Example 3 given further on. Most of these compounds sensitize in the range of 440 to 515 nm.

In a well known type of xerography the photoconductive substances are used in combination with a binding agent the electric specific resistance of which is preferably at least  $10^{10}$  ohm cm.

The quantitative ratio of photoconductive substance to binding agent may vary within wide limits. Preferably the ratio of binding agent to photoconductor is between 1:1 to 1:10 parts by weight. The thickness of the photoconductive layer may be chosen between wide limits according to the requirements of each case. Good recording and reproduction results are attained with electrophotographic layers of a thickness between 1 and 20 $\mu$ , and preferably between 3 and 10 $\mu$ . Too thin layers possess an insufficient insulating power whereas too thick layers require long exposure times.

Suitable binding agents for photoconductive substances of the inorganic type are e.g. described in Belgian patent specifications 612,102 filed Dec. 29, 1961 and 604,126 filed May 24, 1961 both by Gevaert Photo-Producten N.V. The photoconductive recording layers containing photoconductive substances sensitized according to the present invention may further contain photoconductive substances, that cannot be sensitized with the sensitizing compounds corresponding to the above cited general formula e.g. organic monomeric photoconductors described in Belgian patent specifications 585,507 filed Dec. 10, 1959, 585,555 filed Dec. 11, 1959, 587,301 filed Feb. 5, 1960, 585,450 filed Dec. 9, 1959, 587,794 filed Feb. 19, 1960, 589,239 filed Mar. 31, 1960, 594,974 filed Sept. 13, 1960, 595,696 filed Oct. 4, 1960, 597,616 filed Nov. 30, 1960 and 625,683 filed Dec. 5, 1962 all by Gevaert Photo-Producten N.V., and polymeric photoconductors described in Belgian patent specifications 599,627 filed Jan. 30, 1961, 588,049 filed Feb. 26, 1960, 588,048 filed Feb. 26, 1960 and 588,050 filed Feb. 26, 1960 all by

Gevaert Photo-Producten N.V., as well as sensitizers for these photoconductive substances. Furthermore in the recording layer additives known in coating techniques may be used e.g. pigments (see e.g. Belgian patent specification 609,056 filed Oct. 12, 1961 by Gevaert Photo-Producten N.V.), compounds that influence the gloss and/or the viscosity, compounds that counteract ageing and/or oxidation of the layers, compounds that influence the thermal stability of the layers. When selecting any additives preference is given to those that least of all reduce the dark resistivity of the photoconductive layer.

The photoconductive recording layers or sheets sensitized according to the present invention can be prepared by any of the processes known therefor. Thus, the photoconductor-binder composition with a suitable solvent or dispersing liquid for the binder may be coated on a support by a known coating technique e.g. by spraying, by whirling, by dip-coating, or by a coating technique wherein use is made of a doctor blade. The supports or base materials are chosen in view of the particular exposing, recording, developing and/or transfer technique wherein the recording material is to be used.

Preferably for xerographic purposes the support has an electric volume resistivity considerably lower than that of the recording layer. Suitable supports are e.g. described in Belgian patent specifications 602,794 filed Apr. 20, 1961, 612,102 filed Dec. 29, 1961 and 610,060 filed Nov. 8, 1961 all by Gevaert Photo-Producten N.V. and the U.S. patent specification 3,008,825 filed Nov. 20, 1957 by W. G. Van Dorn and O. A. Ullbrich.

The photoconductive layer of an electrophotographic material optically sensitized according to the present invention can be made sensitive for recording purposes by electrically charging according to known methods. The material can, however, also be used in recording techniques, wherein the exposure step precedes charging; for such a technique we refer e.g. to Belgian patent specification 625,335 filed Nov. 27, 1962 by Gevaert Photo-Producten N.V.

The following examples illustrate the present invention without, however, limiting the present invention thereto.

#### EXAMPLE 1

120 g. of copoly(vinyl acetate/vinyl laurate) (80/20) are dissolved in 500 ccs. of toluol. To this solution are added 20 ccs. of a 10% solution in ethanol of mono-octylphosphate and 300 g. of photoconductive zinc oxide (prepared according to the French process) which has been dried for 30 min. on 120° C.

After grinding the whole composition for 15 h. in a ball mill 20 ccs. of a 5% solution in ethanol of succinic acid are added and 6 ccs. of a 10% solution in dimethyl formamide of one of the hydrazone compounds indicated hereinafter in the table. The dispersion obtained is coated on a glassine paper base which does not absorb toluol. The dried layer weighs 25 g. per sq. m.

A series of recording materials are prepared in this way; among this series one material does not contain sensitizing compound and each of the other materials contains a different sensitizing compound as listed hereinafter in the table.

The different recording materials obtained are simultaneously charged with a corona discharging apparatus having a potential difference between the ground and the wires of 6000 v., the wires being connected to the negative pole of a direct current source. The charged materials are exposed under the same conditions with incandescent light bulbs through a grey wedge having a constant 0.1.

The charge images obtained are simultaneously developed with a resin powder toner that contains iron filings as carrier. The toner is fixed by heating.

The sensitometric results presented in the following Table 1 are relative values; the non-sensitized material is given the value 1.

TABLE 1

| List of the sensitizing compound of the list given above | Relative total sensitivity | Maximum spectral sensitivity, nm. |
|----------------------------------------------------------|----------------------------|-----------------------------------|
| 1                                                        | 1                          | 445                               |
| 2                                                        | 5                          | 445                               |
| 3                                                        | 8                          | 505                               |
| 4                                                        | 10                         | 445-505                           |
| 5                                                        | 12                         | 505                               |
| 6                                                        | 10                         | 505                               |

## EXAMPLE 2

250 ccs. of a 20% solution in toluol of silicon resin, 750 ccs. of toluol, 20 ccs. of a 10% solution in ethanol of monobutylphosphate, 300 g. of photoconductive zinc oxide (prepared according to the French process) and 6 g. of the sensitizing compound number 4 are mixed for 16 h. in a ball mill. The further processing steps occur as described in Example 1. The sensitized material has a general sensitivity which is 4 times as high as the sensitivity of the corresponding non-sensitized material.

## EXAMPLE 3

640 g. of copoly(vinyl acetate/vinyl laurate) (80/20) are dissolved in 8 litres of toluol. To this solution are added and mixed therewith in a ball-mill 64 ccs. of a 10% solution in ethanol of monotridecylphosphate and 2.4 kg. of photoconductive zinc oxide (prepared according to the French process).

To the dispersion obtained 320 ccs. of a 5% solution in ethanol of succinic acid are added as well as an amount of a sensitizing compound as listed in the table hereinafter. The further processing occurs as described in Example 1 with a series of recording materials each containing a different sensitizing compound and one material containing no sensitizing compound.

The sensitometric results represented in the following table 2 are also relative values, the non-sensitized material is given the value 1.

TABLE 2

| Percent by weight of sensitizing compound relative to the amount of zinc oxide | Relative total sensitivity | Maximum spectral sensitivity, nm. |
|--------------------------------------------------------------------------------|----------------------------|-----------------------------------|
| 6                                                                              | 20                         | 1                                 |
| 7                                                                              | 64                         | 445-505                           |
| 7                                                                              | 16                         | 445-505                           |
| 8                                                                              | 20                         | 445                               |
| 9                                                                              | 16                         | 505                               |
| 10                                                                             | 16                         | 475                               |
| 11                                                                             | 20                         | 505                               |
| 12                                                                             | 12                         | 515                               |
| 13                                                                             | 20                         | 505                               |
| 14                                                                             | 16                         | 515                               |
| 15                                                                             | 20                         | 515-555                           |
| 16                                                                             | 50                         | 475                               |
| 17                                                                             | 16                         | 445                               |
| 18                                                                             | 20                         | 475                               |
| 19                                                                             | 25                         | 505                               |
| 20                                                                             | 10                         | 505                               |
| 21                                                                             | 5                          | 505-515                           |
| 22                                                                             | 16                         | 515                               |
| 23                                                                             | 64                         | 505                               |
| 24                                                                             | 16                         | 515                               |
| 25                                                                             | 64                         | 505                               |
| 26                                                                             | 40                         | 515                               |
| 27                                                                             | 32                         | 575                               |
| 28                                                                             | 12                         | 505                               |
| 29                                                                             | 16                         | 515                               |
| 30                                                                             | 40                         | 505                               |
| 31                                                                             | 25                         | 505                               |
| 36                                                                             | 25                         | 505                               |
| 38                                                                             | 8                          | 505-515                           |
| 39                                                                             | 6                          | 505-515                           |
| 40                                                                             | 6                          | 505-515                           |
| 41                                                                             | 16                         | 505-515                           |
| 42                                                                             | 64                         | 605                               |
| 43                                                                             | 40                         | 515                               |
| 44                                                                             | 8                          | 605                               |
| 49                                                                             | 16                         | 515                               |
| 56                                                                             | 5                          | 515                               |
| 57                                                                             | 25                         | 605                               |
| 61                                                                             | 8                          | 505                               |
| 62                                                                             | 6                          | 505                               |

## EXAMPLE 4

In the following table the composition of different photoconductive recording layers is illustrated. Said layers are coated on a glassine paper. The relative sensitivity values are calculated by comparing the sensitized materials with the same but non-sensitized material the sensitivity of which is given the relative value 1. The coating and further processing steps of the recording layers are carried out in the same way as illustrated in Example 1.

| Binding agent                                                                                         | Percent by weight of monobutyl phosphate relative to the amount of photoconductive zinc oxide | Ratio by weight of binding agent to photoconductive zinc oxide | Solvent for the binding agent      | Number of the sensitizing compound | Percent by weight of sensitizing compound relative to the amount of zinc oxide | Relative sensitivity | Maximum spectral sensitivity, nm. |
|-------------------------------------------------------------------------------------------------------|-----------------------------------------------------------------------------------------------|----------------------------------------------------------------|------------------------------------|------------------------------------|--------------------------------------------------------------------------------|----------------------|-----------------------------------|
| Polyvinyl butyral                                                                                     | { 0.6<br>0.6<br>0.6 }                                                                         | 2:20                                                           | Ethanol                            | { 6<br>7<br>8 }                    | 0.2<br>0.2<br>0.2                                                              | 3<br>8<br>4          | 445<br>505<br>475                 |
| Copolyester of 2,2-(4,4'-dihydroxy-diphenyl)-propane, isophthalic acid and terephthalic acid (75/25). | { 0.6 }                                                                                       | 4:15                                                           | Methylene chloride.                | { 11<br>9 }                        | 0.2<br>0.2                                                                     | 6<br>12              | 505<br>505                        |
| Copoly(methyl methacrylate/n-butyl methacrylate) (60/40).                                             | 0.6                                                                                           | 10:30                                                          | Acetone                            | 10                                 | 0.1                                                                            | 4                    | 475                               |
| Polycarbonate of 2,2-(4,4'-dihydroxy-diphenyl)-propane.                                               | { 0.6<br>0.6<br>0.6<br>0.6 }                                                                  | 4:15                                                           | Methylene chloride.                | { 8<br>9<br>11<br>9 }              | 0.2<br>0.2<br>0.2<br>0.2                                                       | 12<br>3<br>3<br>3    | 505<br>475<br>505<br>505          |
| Aliphatic keton resin                                                                                 | { 0.6<br>0.6 }                                                                                | 6:15                                                           | Ethanol                            | { 4<br>3 }                         | 2<br>2                                                                         | 16<br>16             | 555<br>505                        |
| Copoly(vinylchloride/vinylacetate/-vinylalcohol) (91/3/6).                                            | { 0.6 }                                                                                       | 4:15                                                           | Acetone                            | 11                                 | 0.2                                                                            | 6                    | 475                               |
| Copoly(n-butyl methacrylate/-isobutylmethacrylate) (40/60).                                           | { 0.6 }                                                                                       | 4:15                                                           | Toluol                             | { 10<br>11<br>9 }                  | 0.2<br>0.2<br>0.2                                                              | 4<br>2.5<br>10       | 475<br>505<br>505-515             |
| Copoly(vinyl acetate/-vinyl stearate) (86/15).                                                        | { 0.6<br>0.6<br>0.6 }                                                                         | 4:22.5                                                         | Ethylene glycol mono methyl ether. | { 10<br>11<br>9 }                  | 0.2<br>0.2<br>0.2                                                              | 20<br>32<br>16       | 475<br>505<br>505                 |
| Copoly(n-butyl methacrylate/-iso-butylmethacrylate) (40/60).                                          | { 0.6<br>0.6 }                                                                                | 4:15                                                           | Toluol                             | { 2<br>3 }                         | 2<br>0.5                                                                       | 16<br>8              | 575<br>445-505                    |

## EXAMPLE 5

To 1 litre of an 8% solution in toluol of copoly(vinyl acetate/vinyl laurate) 80/20) added whilst stirring:

8 ccs. of a 10% solution in ethanol of monobutyl phosphate

300 g. of zinc oxide (prepared according to the French process).

The mixture is ground for 16 h. in a ball mill whereupon 40 ccs. of a 5% solution in ethanol of succinic acid are added. The whole is stirred for another 4 hours and then the dispersion obtained is intimately mixed with the following mixture of optical sensitizing agent:

15 ccs. of a 10% solution in dimethylformamide of hydrazone compound 9 and 3.3 ccs. of 1% solution in dimethyl formamide of Eriocyanine A (Acid Blue 34, C.I. 42,561).

The sensitized composition is coated onto a glassine paper support at a ratio of 30 g. of solid dry substance per sq. m.

The recording layer is successively but separately exposed to a positive colour transparency through a blue, a green and a red filter while before each exposure a uniform electrostatic negative charge is applied to the recording layer by corona discharge. The charge images respectively obtained are developed with a developing pigment dispersed in an insulating liquid (hexane) which pigment has a colour complementary to the colour of the filter used at the exposure. A positive copy of the colour transparency is obtained in this way.

## EXAMPLE 6

Example 2 is repeated but compound 4 is replaced in the same concentration by compound 44.

The sensitized material has a general sensitivity which is 2.5 times as high as the sensitivity of the corresponding non-sensitized material.

## EXAMPLE 7

Example 3 is repeated but using the compounds listed in the table with their sensitometric results.

| Number of the sensitizing compound | Percent by weight of sensitizing compound relative to the amount of zinc oxide | Relative total sensitivity | Maximum spectral sensitivity, nm. |
|------------------------------------|--------------------------------------------------------------------------------|----------------------------|-----------------------------------|
| 44                                 | 0.2                                                                            | 1                          | 605                               |
| 57                                 | 0.2                                                                            | 25                         | 605                               |
| 61                                 | 0.2                                                                            | 8                          | -----                             |
| 62                                 | 0.5                                                                            | 6                          | -----                             |

What is claimed is:

1. A photoconductive recording element comprising a photoconductive layer consisting essentially of photoconductive zinc oxide as the essential photoconductor thereof and a sensitizing amount of a colored chelate complex of an organic chelating agent with ions of said photoconductive zinc oxide, said chelate complex imparting increased light sensitivity to said photoconductive layer, said organic complexing agent having the following general formula:



wherein:

each of Z and Z' represents the necessary atoms for completing a five- or six-membered ring, and

R represents a hydrogen atom or an alkyl radical, said layer being free of sensitizing agents for said photoconductive compound other than said chelate complex.

2. A photoconductive recording element comprising a photoconductive layer consisting essentially of photoconductive zinc oxide as the essential photoconductor

thereof and a sensitizing amount of a colored chelate complex of an organic chelating agent with ions of said photoconductive zinc oxide, said chelate complex imparting increased light sensitivity to said photoconductive layer, said organic complexing agent having the following general formula:



wherein Z' represents the atoms necessary to complete a five- or six-membered ring, said layer being free of sensitizing agents for said photoconductive compound other than said chelate complex.

3. A photoconductive recording element comprising a photoconductive layer consisting essentially of photoconductive zinc oxide as the essential photoconductor thereof and a sensitizing amount of a colored chelate complex of an organic chelating agent with ions of said photoconductive zinc oxide, said chelate complex imparting increased light sensitivity to said photoconductive layer, said organic complexing agent having the following general formula:



wherein Z' represents the atoms necessary to complete a five- or six-membered ring, said layer being free of sensitizing agents for said photoconductive compound other than said chelate complex.

4. A photoconductive recording element comprising a photoconductive layer consisting essentially of photoconductive zinc oxide as the essential photoconductor thereof and a sensitizing amount of a colored chelate complex of an organic chelating agent with ions of said photoconductive zinc oxide, said chelate complex imparting increased light sensitivity to said photoconductive layer, said organic complexing agent having the following general formula:



wherein Z' represents the atoms necessary for completing a five- or six-membered ring, said layer being free of sensitizing agents for said photoconductive compound other than said chelate complex.

5. A photoconductive recording element comprising a photoconductive layer consisting essentially of photoconductive zinc oxide as the essential photoconductor thereof and a sensitizing amount of a colored chelate complex of an organic chelating agent with ions of said photoconductive zinc oxide, said chelate complex imparting increased light sensitivity to said photoconductive layer, said organic complexing agent having the following general formula:



wherein:

each of R<sub>2</sub> and R<sub>3</sub> represents hydrogen, or alkyl, or represent together the atoms necessary to close a homocyclic ring, and

Z' represents the atoms necessary to close a five- or six-membered ring,

said layer being free of sensitizing agents for said photoconductive compound other than said chelate complex.

6. A photoconductive recording element comprising a photoconductive layer consisting essentially of photoconductive zinc oxide as the essential photoconductor thereof and a sensitizing amount of a colored chelate complex of an organic chelating agent with ions of said photoconductive zinc oxide, said chelate complex imparting increased light sensitivity to said photoconductive layer, said organic complexing agent having the following general formula:



wherein:

each of  $\text{R}_4$  and  $\text{R}_5$  represents alkyl or aryl, and  
 $\text{Z}'$  represents the atoms necessary to close a five- or  
six-membered ring,

5 said layer being free of sensitizing agents for said photoconductive compound other than said chelate complex.

#### References Cited

#### UNITED STATES PATENTS

10 3,121,006 2/1964 Middleton et al. ----- 96—1.5  
3,315,599 4/1967 Lind ----- 96—1X

CHARLES E. VAN HORN, Primary Examiner

15 U.S. CL. X.R.

96—1.6, 1.8